

## UNITED STATES PATENT OFFICE

2,532,126

## DIAZOTYPE PHOTOGRAPHIC MATERIAL

Sam Charles Slifkin, Binghamton, and Henry C. Unkauf, Endicott, N. Y., assignors to General Aniline & Film Corporation, New York, N. Y., a corporation of Delaware

No Drawing. Application December 16, 1946,  
Serial No. 716,670

5 Claims. (Cl. 95—6)

1

This invention relates to diazotype photographic materials and more particularly to diazotype layers and compositions designed to yield azo dye images which strongly absorb ultra-violet light normally employed to print material sensitized with diazo compounds.

A primary object of the invention is to produce a diazotype material which will form azo dye images or designs of high actinic opacity and which are readily printable by exposure through ultra-violet light on various diazotype photographic materials. To produce diazotype prints in this manner, it is important that the azo dye images or designs be highly efficient in the absorption of ultra-violet light employed in the printing. The efficacy of such absorption by azo dyes is referred to as actinic opacity. If the actinic opacity is low the images obtained in the print are of poor definition, contrast, and clarity. Heretofore, in order to obtain diazotype layers designed to yield azo dye images of high actinic opacity, it was necessary to employ diazo sensitizers and couplers of relatively high coupling energies and in relatively high concentrations. Such prior art diazotype compositions, however, exhibited two major defects. First, the relatively high coupling energies of the most effective dye formers for this purpose caused premature coupling to occur even during relatively short storage periods of the sensitized materials. Second, attempts to overcome the pre-coupling by stabilizing the components with high concentrations of acidic stabilizing materials caused a rapid degradation of the cellulose fibers composing the base or support carrying the photosensitive layers. This degradation of the cellulose fibers resulted in a rapid loss of physical strength of the papers and particularly exhibited itself by embrittlement of the paper support.

According to our invention, we overcome the drawbacks of the heretofore known procedures by providing a diazotype sensitizing composition in which the component materials possess inherently low coupling energies and require little stabilization by acidic substances. While the actinic opacity of the azo dye formed from such component materials would be expected to be less than with the components heretofore employed, the need for less stabilizing agent and hence reduced alkaline development results in azo images of improved opacity.

Furthermore, our invention makes possible the use of a large excess of a low coupling potential azo component or coupler, thus insuring substantially exclusive formation of the more opaque

2

monoazo dye. It further makes possible, if desired, the use of more diazo salt without excessively decreasing stability (storage life) by mass action. Thus, according to our invention, it is possible to employ high concentrations of the diazo and coupling components without occurrence of excessive premature coupling or without the use of high concentration of acidic stabilizing materials. Cellulosic supports or carriers provided with the light sensitive diazo components of our invention may be stored over longer periods of time without exhibiting the defects and undesirable features of heretofore employed diazo compounds and couplers.

15 Another advantage of our invention is that the solution of the azo components and coupler which we employ may be caused by various mechanical methods to deeply penetrate the support, as for example, by allowing a longer time for the solution to penetrate. This gives added opacity to the azo dye image formed. With the compositions heretofore employed, when deep penetration of the compositions was desired, there was a tendency for the stabilizer to separate from

20 the dye components due to preferential absorption by the support, thereby causing increased pre-coupling of the dye components. On the other hand, our compositions containing components of low coupling potential and small amounts of stabilizers, do not produce such an unfavorable result when applied so as to penetrate deeply into the base or support.

25 According to our invention, we employ as light-sensitive diazo salts, a para-diazo derivative of an N-alkyl- or N-alkylol-m-alkyl, -m-alkoxy, -m-alkylol, or -m-carboxy aniline in combination with a coupler of the following formula:



35 where X may be H,  $-(CH_2)_nCOOH$ , alkyl or alkylol; Y may be H,  $SO_3H$  or a salt thereof, n is a small integer, such as 1, 2, 3 or 4; and Z may be H or a water-solubilizing group obtained by the Mannich reaction, for example,  $-CH_2N(CH_3)_2$ . In Formula I when X is H, Z or Y are other than H.

40 On exposure and development, diazotype layers prepared from such components produce dye images of sepia tones which are highly absorptive

of ultra-violet light. From such azo images or designs there may be then produced through exposure with ultra-violet light prints on various diazotype materials.

In general, the diazo salts which we employ are those from amines of the type which may be represented by the following generic formula:



In the above formula,  $R_1$  is preferably H, but both  $R_1$  and  $R_2$  may be alkyl or alkylol. In the latter case, however, better substantivity results. X is preferably alkyl although it may also be alkoxy, alkylol, or carboxy. More specifically,  $R_1$  is hydrogen, methyl, ethyl, or propyl, hydroxyethyl, or hydroxypropyl;  $R_2$  is ethyl, propyl, butyl, hydroxyethyl or hydroxypropyl; and X is methyl, ethyl, propyl, methoxy, ethoxy, hydroxyethyl, hydroxypropyl or  $\text{--COOH}$ .

The diazo salts can be represented by the following general formula:



In the above formula,  $R_1$ ,  $R_2$  and X have the same significance as in Formula II. The "diazo" radical as employed in the formula and claims stands for a group necessary for the formation of a diazo salt, as for example, diazonium chlorides, carbonates, fluorides and sulfates, and the double salts of diazos with metal halides, such as zinc chloride, boronfluoride, cadmium chloride and tin chloride. The purposes of our invention, however, are not attained by the use of diazo-N-sulfonates, and it is to be understood that the "diazo" radical does not include groups which form diazo-N-sulfonates. As specific examples of the diazonium compounds, there may be mentioned the para-diazonium chloride of N-hydroxyethyl-m-methyl aniline, the p-diazonium zinc chloride double salt of N-ethyl-N-hydroxyethyl-m-methyl aniline, the p-diazonium chloride of N-hydroxypropyl m-ethyl aniline, and the p-diazonium chloride of N-ethyl m-methyl aniline. Instead of the m-alkyl derivatives of the above specified compounds, there may be employed the corresponding m-alkoxy such as the m-methoxy and m-ethoxy derivatives; or the m-alkylol derivatives such as the m-hydroxyethyl and the m-hydroxypropyl derivatives; or the m-carboxy derivatives such as the COOH derivative.

The diazo derivatives may be prepared by diazotizing the corresponding anilines by the well-known diazotizing procedure. For example, the anilines are dissolved in water containing hydrochloric acid and cooled with ice and diazotized with the addition of a slight excess of sodium nitrite. If desired, the diazonium compound which forms can be isolated as the zinc chloride double salt.

As specific examples of the coupler there may

be employed resorcinol-4-sulfonic acid, and its water soluble salts, as for example, its ammonium or sodium salts, 3-hydroxy phenoxyacetic acid, dimethylaminomethyl resorcinol monomethyl ether, and 3-hydroxyphenoxyethyl alcohol.

In practice, the above-mentioned diazo derivatives and coupling compounds are applied in aqueous solution together with stabilizing compounds to a suitable base or support. The compositions may contain one or more of our diazo derivatives together with one or more of the above-mentioned coupling components and may also have present one or more stabilizing compounds, as for example, thiourea, citric acid, boric acid, tartaric and lactic acid, oxalic acid, phosphoric acid, and the like.

If desired, the diazo derivatives and the coupling compounds may be dissolved in separate solutions and applied in sequence to the base or support to be sensitized. In this case, we preferably incorporate the stabilizers in the diazo salt solution. To the solutions there may be added also, if desired, small amounts of wetting or leveling agents or various organic solvents such as ethyl alcohol, acetone, or glycerol.

The concentrations of the diazo derivative and coupling component may vary within a range of about 1-3 moles of coupler per mole of diazo derivative. By permitting the employment of high concentrations of the coupler, our invention insures formation of the more opaque monoazo dye. It is an advantage of our invention that both the diazo compound and the coupler may be utilized in large concentrations without danger of precoupling. In general, the amount of the acid stabilizer is rather small ranging from about 5% to 8% by weight in solution.

The following examples will serve to illustrate our invention. In each, the diazo compound is in the form of its zinc chloride double salt.

#### Example 1

The solution is made up of the following ingredients:

|                                            |       |     |
|--------------------------------------------|-------|-----|
| Water                                      | cc    | 100 |
| Citric acid                                | grams | 5   |
| Glycerol                                   | cc    | 5   |
| Thiourea                                   | grams | 5   |
| Zinc chloride                              | do    | 5   |
| Resorcinol-4-sulfonic acid                 | do    | 4   |
| p-Diazo of N-hydroxyethyl-m-methyl aniline | grams | 4   |

The solution is applied, for example, in excess to one side of a well-sized lightweight paper. The excess is removed by a doctor blade and the sensitive layer then formed on the paper is dried with warm air. After drying, the sensitized paper is exposed to ultra-violet rays through a design. A sepia colored dye image is formed on development in an atmosphere of ammonia. The dye image thus obtained is highly absorptive of ultra-violet light and may be employed as a pattern for producing additional prints on diazotype paper by exposure to ultra-violet light.

#### Example 2

A sensitizing solution was made up of the following ingredients:

|             |       |     |
|-------------|-------|-----|
| Water       | cc    | 100 |
| Citric acid | grams | 5   |
| Boric acid  | do    | 2   |
| Thiourea    | do    | 5   |
| Glycerol    | cc    | 5   |

|                                                            |       |   |
|------------------------------------------------------------|-------|---|
| Zinc chloride                                              | grams | 5 |
| 3-hydroxyphenoxy acetic acid                               | do    | 3 |
| p-Diazo of N-ethyl - N - hydroxyethyl - m - methyl aniline | grams | 4 |

This solution was employed to impregnate a piece of well-sized, light weight paper and the excess solution was removed, after which the paper was dried. The dried, sensitized paper was then exposed as in Example 1. A sepia toned dye image of high actinic opacity was formed.

#### Example 3

A sensitizing solution was prepared from the following ingredients:

|                                                 |       |     |
|-------------------------------------------------|-------|-----|
| Water                                           | cc    | 100 |
| Citric acid                                     | grams | 5   |
| Thiourea                                        | do    | 5   |
| Glycerol                                        | cc    | 5   |
| Zinc chloride                                   | grams | 5   |
| Dimethylaminomethyl resorcinol monomethyl ether | grams | 3   |
| p-Diazo of N-hydroxypropyl-m-methyl aniline     | grams | 4   |

This solution on application to a paper base, formed a sensitized layer which when exposed and developed as described in the previous examples formed sepia tone dye images which were highly opaque to actinic rays.

#### Example 4

A piece of light weight, well-sized paper was sensitized, exposed and developed as described in the previous example except that the sensitized layer on the paper was formed from the following solution. A sepia azo dye image of high actinic opacity was obtained.

|                                                 |       |     |
|-------------------------------------------------|-------|-----|
| Water                                           | cc    | 100 |
| Citric acid                                     | grams | 6   |
| Boric acid                                      | do    | 2   |
| Thiourea                                        | do    | 5   |
| Glycerol                                        | cc    | 5   |
| Zinc chloride                                   | grams | 5   |
| Dimethylaminomethyl resorcinol monomethyl ether | grams | 2   |
| p-Diazo of N-ethyl-m-methyl aniline             | do    | 4   |

If desired, a small amount of resorcinol ranging from about 0.5-1% may be added to the solutions in order to shade the sepia dye image obtained.

The above examples are merely illustrative of our invention and we have found that other diazo compounds coming under the general Formula III, and other couplers coming under the general Formula I are useful in our process. However, we prefer those diazo derivatives where  $X$  is an alkyl,  $R_1$  is H and  $R_2$  is an alkylol since they have the lowest coupling potentials and exhibit greatest substantivity toward the support. Accordingly, we prefer to employ the p-diazo derivatives of a mono-N-alkylol-m-alkyl aniline.

In place of paper as the support or base for carrying the light-sensitive layers, there may also be employed sheets or films, for example, those prepared from cellulose acetate, cellulose nitrate, regenerated cellulose and the like; cloth or glass. The sensitizing preparations may be applied to the base or support by dipping, spraying, coating, brushing, or by other ways known to those skilled in the art.

The diazotype copying materials herein described exhibit excellent keeping qualities. They can be stored over long periods without degrada-

tion of the paper base or premature coupling of the components. This together with the high stability of the azo components, their low coupling energies and the production of azo dyes of high actinic opacity are among the advantageous features of our invention.

We claim:

1. A diazotype photographic material comprising a light-sensitive para-diazo compound of the following formula:



15 where  $R_1$  represents a member selected from the group consisting of hydrogen, an alkyl group and an alkylol group;  $R_2$  represents a member selected from the group consisting of an alkyl group and an alkylol group;  $X$  represents a member selected from the group consisting of an alkyl group, an alkoxy group, an alkylol group, and a carboxy group; and a coupler of the following general formula:



20 where  $X$  represents a member selected from the group consisting of hydrogen,  $-(CH_2)_nCOOH$ , alkyl and alkylol groups,  $n$  being a small number; 40  $Y$  is selected from the group consisting of hydrogen and  $-SO_3H$  and a salt thereof;  $Z$  is selected from the group consisting of hydrogen and an aminomethyl group and wherein when  $X$  is hydrogen at least one of  $Y$  and  $Z$  is other than 45 hydrogen in the proportion of about 1 to 3 mols of coupler to 1 mol of diazo compound.

2. A diazotype paper having a light-sensitive layer comprising a light-sensitive para-diazo compound of the following formula:



50 where  $R_1$  represents a member selected from the group consisting of hydrogen, an alkyl group and an alkylol group;  $R_2$  represents a member selected from the group consisting of an alkyl group and an alkylol group;  $X$  represents a member selected from the group consisting of an alkyl group, an alkoxy group, an alkylol group, and a carboxy group; and a coupler of the following general formula:



where  $X$  represents a member selected from the group consisting of hydrogen,  $-(CH_2)_nCOOH$ , alkyl and alkyol groups,  $n$  being a small number;  $Y$  is selected from the group consisting of hydrogen and  $-SO_3H$  and a salt thereof;  $Z$  is selected from the group consisting of hydrogen and an aminomethyl group and wherein when  $X$  is hydrogen at least one of  $Y$  and  $Z$  is other than hydrogen in the proportion of about 1 to 3 mols of coupler to 1 mol of diazo compound. 10

3. A diazotype paper having a light-sensitive layer comprising para-diazo-N-hydroxyethyl-methyl aniline and resorcinol-4-sulfonic acid in the molecular proportion of 1:2. 15

4. A diazotype paper having a light-sensitive layer comprising para-diazo-N-ethyl-N-hydroxyethyl-m-methyl aniline and 3-hydroxy phenoxyacetic acid in the molecular proportion of 1:1. 15

5. A diazotype paper having a light-sensitive layer comprising para-diazo-N-hydroxypropyl-m- 20

ethylaniline and dimethylaminomethyl resorcinol monomethyl ether in the molecular proportion of 1:2.

SAM CHARLES SLIFKIN.  
HENRY C. UNKAUF.

#### REFERENCES CITED

The following references are of record in the file of this patent:

#### UNITED STATES PATENTS

| Number    | Name           | Date          |
|-----------|----------------|---------------|
| 1,628,279 | Krieger        | May 10, 1927  |
| 1,807,761 | Sprongerts     | June 2, 1931  |
| 1,821,306 | Hingst         | Sept. 1, 1931 |
| 1,989,065 | Schmidt et al. | Jan. 22, 1935 |
| 2,196,950 | Zahn           | Apr. 9, 1940  |
| 2,245,628 | Poser          | June 17, 1941 |
| 2,246,425 | Poser et al.   | June 17, 1941 |
| 2,437,868 | Glahn et al.   | Mar. 16, 1948 |